

1

3,297,437

**COPPER BASE ALLOYS CONTAINING  
MANGANESE AND ALUMINIUM**

Leendert Bosman, Drunen, Netherlands, assignor to Lips N.V., Drunen, Netherlands, a corporation of the Netherlands

No Drawing. Filed Jan. 27, 1964, Ser. No. 340,515  
Claims priority, application Netherlands, Feb. 13, 1963,  
288,920

4 Claims. (Cl. 75—157.5)

This invention relates to copper base alloys containing manganese and aluminium, and to shaped articles, manufactured from such alloys.

It is known to have an alloy consist of 1 to 5% iron, 1 to 6% nickel, 6 to 9% aluminium, 10 to 15% manganese and as balance substantially copper. Moreover, a monophase forging alloy is known, containing less than 5% iron, less than 6% nickel, between 5 and 20% manganese, 1 to 7% aluminium and 0.01 to 0.2% arsenic, antimony or phosphorus, balance copper. The arsenic, antimony or phosphorus increase the corrosion resistance by preventing the aluminium from being extracted from the alloy. Such known alloys particularly have a composition of between 5 and 13% of manganese and experiments have been made with an alloy of 12% manganese.

Moreover, an alloy is known having 8.5% to 10% manganese, 8.5 to 10.5% aluminium, 2.5 to 5% iron, 2 to 3% nickel, less than 0.25% impurities such as zinc, lead and silicon, and the balance copper. Such alloys have a good resistance against corrosion and cavitation-erosion-corrosion in seawater.

This invention is based upon the discovery that the corrosion resistance and particularly the resistance against cavitation-erosion-corrosion of such alloys in seawater, particularly at high relative water speeds, may be improved at such known manganese contents (about 10 to 16%) while maintaining good mechanical characteristics such as tensile strength, 0.2-yield limit, total elongation, contraction at rupture and fatigue strength under rotated bending both in air and in seawater, without increase of melting point, and while maintaining a good weldability, deformability in hot condition and extrudability if such an alloy is manufactured with the following composition:

|                                                           | Percent  |
|-----------------------------------------------------------|----------|
| Iron                                                      | 1 to 9   |
| Nickel, if desired entirely or in part replaced by cobalt | 0 to 7   |
| Aluminium                                                 | 3 to 9   |
| Nickel and iron together                                  | 3 to 14  |
| Manganese                                                 | 10 to 16 |
| Zinc                                                      | 1 to 7   |
| Balance copper and usual impurities                       |          |

It has moreover appeared in this respect that zinc is able to replace part of the aluminium in its influence on the mechanical characteristics and on the precipitation of the iron-rich phase during solidification of the molten alloy, which influences the corrosion resistance. This means that during the manufacture of the molten bath of the alloy not only aluminium (and if desired manganese) but also zinc may be used to correct the conditions and the composition and finally the characteristics of the alloy. This facilitates manufacture. The influence of aluminium is so pronounced that the aluminium percentage is highly critical and small, possibly unintentional deviations of the aluminium content have a high influence. Zinc is less critical in this respect.

It has appeared that zinc has a so-called aluminium equivalent of about 0.3 to 0.4. It appears therefrom that

2

much more zinc could be added without great changes in characteristics than aluminium would entrain.

Zinc has a much lower melting point than manganese, which has lower aluminium equivalent than zinc, namely about 0.1 to 0.2. Thus less zinc than manganese is necessary for the same effect and zinc is not only more economical than manganese, but due to the low melting point of zinc it is possible to produce the melt more rapidly and with less heating energy, particularly with respect to final corrections of the bath.

The surprising character of the present invention appears from the fact that up to now in comparable alloys with relatively high manganese content no zinc was used at all, such as in the alloy given above with 1 to 5% iron,

1 to 6% nickel, 6 to 9% aluminium, 10 to 15% manganese, balance copper. In the publication of the British Standards Institution: B.S. 1400: 1961: Schedule of Copper Alloy Ingots and Copper Alloy Castings, pages 65-68 for manganese-aluminium-copper alloys, to total absence of zinc is taken as a basis.

The invention will now further be explained on the basis of the following examples:

*Example I.*—The following elements were melted together in a suitable furnace:

|                                      | Percent |
|--------------------------------------|---------|
| Iron                                 | 6.6     |
| Nickel                               | 2.7     |
| Aluminium                            | 6.7     |
| Manganese                            | 11.7    |
| Zinc                                 | 1.8     |
| Balance copper and usual impurities. |         |

The alloy was cast in a sand mold bonded by cement. Examination of a sample of this alloy gave the following values:

|                        |               |
|------------------------|---------------|
| Tensile strength       | 95,000 p.s.i. |
| Elongation at rupture  | 30% (1/d=5).  |
| Contraction at rupture | 34.4%         |

*Example II.*—In a suitable furnace an alloy was made which obtained the following composition:

|                                      | Percent |
|--------------------------------------|---------|
| Iron                                 | 6.0     |
| Nickel                               | 2.7     |
| Aluminium                            | 6.4     |
| Manganese                            | 12.2    |
| Zinc                                 | 5.2     |
| Balance copper and usual impurities. |         |

A sample gave:

|                       |                |
|-----------------------|----------------|
| Tensile strength      | 103,000 p.s.i. |
| Elongation at rupture | 25.5% (1/d=5). |

*Example III.*—An alloy was made with the following composition:

|                                      | Percent |
|--------------------------------------|---------|
| Iron                                 | 3.2     |
| Nickel                               | 2.7     |
| Aluminium                            | 8.1     |
| Manganese                            | 11.9    |
| Zinc                                 | 3.6     |
| Balance copper and usual impurities. |         |

A sample was tested and gave the following results:

|                        |                |
|------------------------|----------------|
| Tensile strength       | 115,000 p.s.i. |
| Elongation at rupture  | 19.5% (1/d=5). |
| Contraction at rupture | 17%.           |

*Example IV.*—An alloy was made with the following composition:

|                                      | Percent |
|--------------------------------------|---------|
| Iron                                 | 6.8     |
| Nickel                               | 0.14    |
| Aluminium                            | 7.1     |
| Manganese                            | 10.8    |
| Zinc                                 | 4.9     |
| Balance copper and usual impurities. |         |

A sample gave:

|                        |               |
|------------------------|---------------|
| Tensile strength       | 97,000 p.s.i. |
| Elongation at rupture  | 30% (1/d=5).  |
| Contraction at rupture | 38%.          |

*Example V.*—An alloy was made with the following composition:

|                                      | Percent |
|--------------------------------------|---------|
| Iron                                 | 6.6     |
| Nickel                               | 5.0     |
| Aluminium                            | 5.8     |
| Manganese                            | 15.4    |
| Zinc                                 | 4.3     |
| Balance copper and usual impurities. |         |

A sample gave:

|                        |                |
|------------------------|----------------|
| Tensile strength       | 103,000 p.s.i. |
| Elongation at rupture  | 16% (1/d=5).   |
| Contraction at rupture | 15.4%.         |

*Example VI.*—An alloy was made with the following composition:

|                                      | Percent |
|--------------------------------------|---------|
| Iron                                 | 6.5     |
| Nickel                               | 2.7     |
| Aluminium                            | 6.5     |
| Manganese                            | 11.5    |
| Zinc                                 | 4.1     |
| Balance copper and usual impurities. |         |

Testing of a sample gave the following results:

|                       |               |
|-----------------------|---------------|
| Tensile strength      | 97,000 p.s.i. |
| 0.2 yield limit       | 42,000 p.s.i. |
| Elongation at rupture | 25% (1/d=5).  |

This alloy was with respect to its corrosion resistance and cavitation-erosion-corrosion resistance in seawater at a speed of 125 feet per second compared with the following known manganese-aluminium-cooper alloy: iron 2.74%, nickel 2.03%, aluminium 8.45%, manganese 12.04%, balance copper and impurities.

|                       |                |
|-----------------------|----------------|
| Aluminium equivalent  | 10.25.         |
| Tensile strength      | 97,500 p.s.i.  |
| 0.2 yield limit       | 44,000 p.s.i.  |
| Elongation at rupture | 18.3% (1/d=5). |

It appeared from the comparison that the corrosion resistance of the alloy according to the invention, Example VI, was about 60% higher than of said known alloy. The cavitation-erosion-corrosion resistance was about 100% better than of said known alloy.

*Example VII.*—An alloy was made with the following composition:

|                                      | Percent |
|--------------------------------------|---------|
| Iron                                 | 2.7     |
| Nickel                               | 2.9     |
| Aluminium                            | 6.7     |
| Manganese                            | 12.2    |
| Zinc                                 | 4.4     |
| Balance copper and usual impurities. |         |

Testing of a sample gave:

|                       |                             |
|-----------------------|-----------------------------|
| Tensile strength      | 72.6 kg./mm. <sup>2</sup> . |
| 0.2 yield limit       | 31.7 kg./mm. <sup>2</sup> . |
| Elongation at rupture | 22.9% (1/d=5).              |

The alloy was tested as indicated under Example VI and compared with the known alloy given in said example. The corrosion-resistance of the alloy according to the invention was about 15% better than of said known alloy. The cavitation-erosion-corrosion resistance was also in this case about 100% better than of said known alloy.

The alloy of Example VII was extruded and a sample of said extruded alloy had a tensile strength of 92,500 p.s.i., a 0.2 yield limit of 60,000 p.s.i. and an elongation at rupture of 32% (1/d=5).

*Example VIII.*—An alloy was made with the following composition:

|                                | Percent |
|--------------------------------|---------|
| Iron                           | 4.5     |
| Nickel                         | 2.1     |
| Cobalt                         | 0.8     |
| Aluminium                      | 6.4     |
| Manganese                      | 12.1    |
| Zinc                           | 4.9     |
| Balance copper and impurities. |         |

Testing of a sample thereof gave:

|                       |                |
|-----------------------|----------------|
| Tensile strength      | 102,000 p.s.i. |
| Elongation at rupture | 26.5% (1/d=5). |

All percentages of alloy components given in this specification and in the attached claims relate to percentages by weight.

What we claim is:

1. An alloy having the following weight composition: 1 to 9% iron, up to 7% of a member selected from the class consisting of nickel, cobalt, and mixtures thereof, 3 to 9% aluminum, 10 to 16% manganese, 1 to 7% zinc, balance essentially copper, the sum of the iron and any nickel being 3 to 14%, in which the aluminum equivalent, calculated by adding to the aluminum percentage 0.15 times the manganese percentage and 0.35 times the zinc percentage, is between 7 and 13.
2. An alloy as claimed in claim 1, in which the aluminum equivalent is between 9 and 11.5.
3. An alloy having the following weight composition: 2 to 7% iron, 1 to 5% of a member selected from the class consisting of nickel, cobalt, and mixtures thereof, 5 to 8% aluminum, 10 to 16% manganese, 1.6 to 5.5% zinc, balance essentially copper, in which the aluminum equivalent, calculated by adding to the aluminum percentage 0.15 times the manganese percentage and 0.35 times the zinc percentage, is between 7 and 13.
4. An alloy as claimed in claim 3, in which the aluminum equivalent is between 9 and 11.5.

#### References Cited by the Examiner

##### UNITED STATES PATENTS

|           |        |                  |          |
|-----------|--------|------------------|----------|
| 2,085,416 | 6/1937 | Corson           | 75—157.5 |
| 2,372,152 | 3/1945 | Whittaker et al. | 75—157.5 |
| 3,134,669 | 5/1964 | Putter et al.    | 75—161   |

##### FOREIGN PATENTS

|         |         |                |
|---------|---------|----------------|
| 880,325 | 12/1942 | France.        |
| 762,235 | 11/1956 | Great Britain. |
| 868,276 | 5/1961  | Great Britain. |

DAVID L. RECK, Primary Examiner.

C. N. LOVELL, Assistant Examiner.